

Nov. 2, 1937.

J. L. SCHUELER

2,097,472

PROCESS OF FLAME TREATING COATED MATERIALS

Filed Oct. 4, 1934



Inventor:  
Julian L. Schueler,  
By Banning & Banning  
Attns.

## UNITED STATES PATENT OFFICE

2,097,472

## PROCESS OF FLAME TREATING COATED MATERIALS

Julian L. Schueler, Kokomo, Ind., assignor, by mesne assignments, to C. W. La Porte, Peoria, Ill., and J. L. Schueler, Kokomo, Ind., trustees

Application October 4, 1934, Serial No. 746,859

5 Claims. (Cl. 91—59.1)

This invention relates to a process for the treatment of coated iron and steel materials. It is applicable particularly to coated wires, round, flat, shaped, strips, etc., whether or not they be intended for fabrication. In the ensuing description, the invention will be explained, by way of example, with reference to wires coated with zinc, although possibly it may be used to advantage with coatings other than zinc applied to iron and steel materials in form other than wire.

It is a primary object of my invention to treat the material upon which the coating is still molten, by flames in such a manner as to promote an even distribution of the coating over the material, to render the coating more smooth and even, and otherwise to impart a beneficial effect to the coating. These and other objects are attained by the application of flames to the coated material for a period of time and under conditions of temperature, all as hereinafter set out. An apparatus suitable for this purpose is illustrated in the accompanying drawing wherein is shown a number of wires emerging from a coating bath to travel in parallelism through a flame wave which is shown as undulating between upper and lower deflecting surfaces illustrated in vertical section to better exhibit the construction.

In carrying out this invention, particularly in the case of wires, I utilize a pan P in which is contained a bath B of molten zinc at a suitable galvanizing temperature, perhaps about 860 degrees F. Through this bath may be drawn a number of wires w in parallelism. Immediately upon leaving the bath, each wire is taken through a coating regulator R which removes dross, skimmings, and grosser articles, and also reduces the amount of coating remaining on the wire to a point at which a beneficial treatment by flames may be practiced. The weight of coating material so removed from each wire may perhaps be 50% or more, the amount being subject to the setting of the regulator.

Upon leaving the coating regulators the wires travel side by side through a flame apparatus which may comprise upper and lower deflector surfaces U and L, respectively. By preference, these surfaces are sloped upwardly very slightly, as shown in the drawing. These deflector surfaces which desirably are constituted by refractory blocks define a space which is open on all sides, and by preference approach each other toward the end from which the wires emerge to pass on through an air cooling space preliminary to being guided by rollers G on their way to take-up reels. The upper and lower deflector surfaces

are adjustable relative to each other, so that the space between them may be varied as desired.

Projected from a line of burner openings O into the space from the end thereof which is proximate to the bath is a waving flame sheet F which, as shown, proceeds downwardly and forwardly from the upper deflector surface to strike the lower deflector surface, and then rebound therefrom, and again rebound from the upper deflector surface, and so on throughout the length of the flame apparatus. The flame sheet which thus undulates throughout the space between the two deflector surfaces is impinged against the several wires on all sides thereof during their travel through the flame apparatus. Further description of the apparatus per se need not be given here inasmuch as a full explanation thereof appears in my Reissue Patent No. 19,209 dated June 12, 1934.

It is my experience in the flame treating of zinc coated wire that very satisfactory results may be obtained with certain changing temperature conditions for a brief interval of time. It is accordingly with this aspect of my invention that the following description is particularly concerned.

I find it advantageous to utilize a flame apparatus in which may be maintained a continuous elongated flame sheet of between eight and eleven feet in length. The flame sheet so projected is confined practically, if not entirely, within the space defined between the upper and lower deflector surfaces which accordingly may be of substantially the same length. In practice, these surfaces radiate considerable heat which augments that of the flame sheet which latter, however, is alone responsible for the smoothing and evening of the metallic coating so treated.

It is desirable that a temperature of from 2000 degrees F. to 2400 degrees F. should obtain at the point where the waving flame sheet first strikes the deflector surfaces. At the exit end of the apparatus, this temperature is, by preference, much lower, perhaps around 1700 degrees F. Accordingly, there may be a differential range of three to seven hundred degrees F. between the two ends of the flame sheet, the point of highest temperature being adjacent the burners from which the flames are projected.

Between the length of the flame, the temperature of the flame, the speed of wire travel through the flame, and also the gauge of the wire itself, there is a close relationship which determines the character of the result produced by the present flame treatment. As to the speed of wire travel and its consequent duration of treatment by the flame, the following is noted:

According to my process, it is feasible to galvanize concurrently a number of wires varying widely in size, and also to treat successfully all such wires by a flame apparatus such as hereinbefore described. The speed of travel for 9 gauge wire (.1485 inch diameter) may in commercial practice be about sixty-seven feet per minute, although I have obtained successful results with a higher speed of from ninety to one hundred feet per minute. For a 15½ gauge wire a commercial speed would be about one hundred fifty seven feet per minute. At the lower of these movement rates, the 9 gauge wire would travel through a flame zone of ten and one-half feet for approximately nine seconds, and the 15½ gauge wire for approximately four seconds. At higher speeds the wire will be subjected to flame treatment for a correspondingly shorter time. It is accordingly optional, within a fairly wide range, as to the speed of wire travel and the period of flame treatment that may be selected.

I have ascertained that a very beneficial effect results from the action of flames on a molten coating of material, such as zinc, applied to a base, such as iron or steel. It is not the temperature per se which is responsible for the better distribution of the coating over the base to which it is applied, nor for the improved evenness and smoothing of the coating which is conducive to enhanced ductility and adherence. Rather it is the flame action itself, due perhaps to its impingement upon the coating. The effect of the flame is satisfactory when it is applied at temperatures within the range above suggested, and also when the temperature conditions are such that there is a progressive decrease in the temperature during the period of flame treatment.

From the foregoing description it is manifest that flexibility characterizes the operating conditions surrounding a successful flame treatment such as this invention is concerned with. Although these conditions may be varied considerably, as above indicated, I regard it as important that the flame temperature be highest at or near the initial moment of treatment, and that this temperature be substantially reduced at or near the final moment of treatment.

I claim:

1. The process of treating metal coated materials having an iron base to produce a coating of superior smoothness and evenness which comprises moving such materials at a speed depend-

ent upon the thickness of such materials through a zone of flame treatment of predetermined length wherein the temperature of the flame treatment is progressively decreased in the direction of movement of such materials through a range of between 2400° F. and 1700° F.

2. The process of galvanizing wire to produce a galvanizing coating of superior smoothness and evenness which comprises moving a wire on which is a molten zinc coating, for a period ranging between three and ten seconds, through a flame treating zone wherein are maintained progressively decreasing temperatures ranging between 2400° F. and 1700° F., the wire being required to encounter the point of maximum temperature first.

3. A step in the process of galvanizing wire which consists in moving the wire upon which a zinc coating is still molten through a zone of flames ranging between eight and eleven feet at a speed ranging between fifty and two hundred feet per minute, the flame temperatures ranging between 2400° F. and 1700° F. from one end of said zone to the other.

4. The process of treating metal coated materials having an iron base to produce a coating of superior smoothness and evenness, which comprises moving the base upon which the coating is in molten state through a zone of flame treatment of predetermined length and at a speed dependent upon the character of the coating material, and progressively reducing by a differential range of 300 to 700 degrees F. the temperature of the flame treatment in the direction of movement of the coated base, the lower limit of said range being above the melting point of said coating material.

5. The process of treating metal coated materials having an iron base to produce a coating of superior smoothness and evenness, which comprises regulating the weight of coating upon the base, moving such regulated coated base throughout a flame treating zone of predetermined length and at a speed dependent upon the weight of coating material on said base, and progressively reducing by a differential range of 300 to 700 degrees F. the temperature of flame treatment in the direction of movement of the coated base, the lower limit of said range being above the melting point of said coating material.

JULIAN L. SCHUELER.